

## UNITED STATES PATENT OFFICE

2,636,878

METHOD OF MAKING TEXTILE FIBER  
DRAFTING ELEMENTS

Richard A. Garrett, Lancaster Township, Lancaster County, Pa., assignor to Armstrong Cork Company, Lancaster, Pa., a corporation of Pennsylvania

No Drawing. Application September 29, 1950,  
Serial No. 187,669. In Great Britain November  
11, 1949

4 Claims. (Cl. 260—83.3)

1

This invention relates to a method of making textile fiber drafting elements and is concerned particularly with the production of roll covers or cots which are used in the drafting of cotton, rayon, worsted, and other fibers. Such cots are manufactured with a matrix of synthetic rubber and may include cork particles and other compounding ingredients. In the drafting of fibers, it has been found that a tendency exists for the fibers to "lap up" around the drafting roll, and the problem is particularly difficult in drafting rayon and similar fibers. This "lapping" tendency is present in roll covers formed from certain types of butadiene-acrylonitrile synthetic rubbers, such as the synthetic rubber of this type sold as "Perbunan" or "Paracril." This product is made by Standard Oil Company of New Jersey and contains 74% butadiene and 26% acrylonitrile. Other examples of butadiene-acrylonitrile synthetic rubbers which are deficient in lap resistance are two varieties of "Hycar" made by Goodrich Chemical Company and known as "O. R. 15" which contains 60% butadiene and 40% acrylonitrile and "O. R. 25" which contains 75% butadiene and 25% acrylonitrile, and certain varieties of "Chemigum" manufactured by Goodyear Tire and Rubber Company, known as "Chemigum N-3" which contains 60% butadiene and 40% acrylonitrile and "Chemigum N-4" which contains 70% butadiene and 30% acrylonitrile.

The principal object of the present invention is to improve the lap resistance of textile fiber drafting elements such as roll covers which employ a matrix of butadiene-acrylonitrile synthetic rubber which is normally deficient in lap resistance.

According to the present invention, the deficient synthetic rubber in an un compounded condition is heated in the presence of oxygen while it is mechanically worked to expose substantially all of it to oxygen while in a heated condition for an interval sufficient to substantially improve the lap resistance of the synthetic rubber. Thereafter, the rubber is compounded and vulcanized in the usual manner.

As disclosed in Patents 2,450,409 and 2,450,410, the lap resistance of various synthetic rubbers can be improved by adding animal glue or other electrolyte thereto, and the present invention may be used in the preparation of roll covers with or without the addition of electrolytes.

The temperature and the duration of the heat treatment vary over very wide ranges, depending upon the particular synthetic rubber being treat-

2

ed, the type of mechanical working, the presence of anti-oxidants in the un compounded synthetic rubber stock, and other variable factors. The interval of treatment will depend, in addition to the temperature to which the stock is elevated during mechanical working, higher temperatures normally requiring shorter periods of time to effect the desired improvement in lap resistance. Overtreatment by excessive heating or from heating for a prolonged period results in a noticeable decrease in lap resistance and also tends to produce compounds which are difficult to process because of increase in the "nerve" of the compound. Charring of the rubber or other deleterious action may also result from overtreatment. Also, as the temperature is increased the duration of the treatment decreases and becomes more difficult to control because the time factor is so short. It is preferred, therefore, to heat at temperatures below the critical upper limit and for a fairly substantial period of time to obtain optimum lap resistance and avoid deleterious action upon the synthetic rubber, at the same time providing for convenient control of the process. The temperature must be elevated substantially above normal mixing or milling temperatures in order to secure maximum lap resistance. The lower the temperature, generally, the longer the treatment period required to obtain maximum results.

The heat treatment effect is believed to be a combination time-and-temperature action; and there is believed to be some oxidation or other chemical reaction involved, for heat treatment in the absence of oxygen does not improve lap resistance of the synthetic rubber when compounded. It has been observed that the use of anti-oxidants beyond the normal small amount of anti-oxidant contained in the un compounded synthetic rubber as supplied by the manufacturer tends to inhibit the effect of the heat treatment.

The heat treatment may be effected by processing the un compounded synthetic rubber in a heated Banbury mixer or a heated two-roll rubber mill. As mentioned previously, a factor affecting the final lap resistance of the product is the nature of the mechanical working or mastication of the un compounded synthetic rubber. The results achieved by mechanically working on an open two-roll rubber mill will differ from those achieved by mastication in a Banbury mixer using the same temperature and period of treatment. It is believed that this difference may be due to the accessibility of the material to oxygen during the course of the mastication, this, of

course, being different in the case of the open mill than in a closed Banbury mixer.

The mechanical working should be accomplished for a period of time sufficient to expose substantially all of the synthetic rubber to oxygen while in a heated condition. Where there is subsequent mechanical working of the mass at a high temperature; for example, when an electrolyte such as glue is mixed into the synthetic rubber, as disclosed in the patents mentioned, it will not be necessary for the original heat treatment to be as extensive as in the case where there is no subsequent high temperature working of the mass.

The maximum temperature of treatment of butadiene-acrylonitrile synthetic rubber on a commercial scale is about 375° F., and the minimum interval of treatment is about five minutes. The minimum temperature is about 250° F. for commercial production, and the maximum interval is about fifty minutes. These times and intervals of treatment will vary, as mentioned above.

The following are examples of the heat treatment of a "Perbunan" or "Paracril" stock of uncompounded rubber in accordance with the present invention:

|                                                                                                                                          | Time and Temperature<br>Mastication | Type of<br>Mastication | Subsequent Milling for<br>Addition of Glue | Lap Resistance of Cot    |
|------------------------------------------------------------------------------------------------------------------------------------------|-------------------------------------|------------------------|--------------------------------------------|--------------------------|
| 1                                                                                                                                        | 50 minutes at 250° F.               | open mill              | 10-15 minutes at 240° F.                   | Substantial improvement. |
| 2                                                                                                                                        | 10 minutes at 275° F.               | do                     | do                                         | Do.                      |
| 3                                                                                                                                        | 25 minutes at 275° F.               | do                     | do                                         | Maximum improvement.     |
| 4                                                                                                                                        | 25 minutes at 320° F.               | do                     | none                                       | Do.                      |
| (This example shows that a more extensive original heat treatment is desirable if there is no subsequent high temperature milling step.) |                                     |                        |                                            |                          |
| 5                                                                                                                                        | 25 minutes at 275° F.               | Banbury mixer          | 10-15 minutes at 240° F.                   | Slight improvement.      |
| 6                                                                                                                                        | 25 minutes at 320° F.               | do                     | do                                         | Maximum improvement.     |

(Longer times and higher temperatures than indicated above for maximum lap resistance tend to make the material less readily workable.)

The preferred temperature range is between about 250° F. and about 320° F., and the preferred interval of treatment is about twenty-five minutes. This provides a temperature range which is low enough to permit accurate control of the process. It also provides a reasonably short period of treatment which will not be burdensome in commercial practice. Where an open mill is employed, the optimum results appear to be achieved by heating at 275° F. for twenty-five minutes where there is subsequent milling for the addition of glue in the compounding of the stock. Where there is no subsequent high temperature milling, the heat treating of the uncompounded stock is effected at about 320° F. for optimum results. Where Banbury mixing is employed to effect the mechanical working of the uncompounded synthetic rubber, optimum results are achieved at 320° F., with a treating interval of twenty-five minutes where there is a subsequent milling for the addition of glue in the compounding of the stock.

Where it is possible to elevate the temperature of the mill rolls by the application of high pressure steam, temperatures in the order of 375° F. may be employed for a period of about five minutes. As mentioned above, when higher temperatures are employed, care must be exercised to avoid overtreatment.

The synthetic rubber which has been heat treated in accordance with the invention may be compounded with the usual ingredients, including an electrolyte such as glue, if desired,

to form roll covers and other textile fiber drafting elements. A specific example of a roll cover compound produced in accordance with the invention for fabrication into a cot or roll covering is given below:

|                                                                                              | Parts by weight |
|----------------------------------------------------------------------------------------------|-----------------|
| "Perbunan" (butadiene-acrylonitrile copolymer) heat treated in accordance with the invention | 100             |
| 10 Sulphur                                                                                   | 10              |
| Triacetin                                                                                    | 10              |
| Titanium dioxide                                                                             | 15              |
| Zinc oxide                                                                                   | 10              |
| Graphite No. 64                                                                              | 2.6             |
| 15 Benzothiazyl disulphide                                                                   | 1.5             |
| Diphenylguanidine                                                                            | 0.2             |
| Glue                                                                                         | 50              |

The "Perbunan" in the above example is prepared by heat treatment in an open two-roll rubber mill for twenty-five minutes at 275° F. Into this heat-treated "Perbunan" is dispersed the glue which has been water-softened and the mixture is milled for ten-fifteen minutes at about 240° F. to drive off the moisture and obtain a uniform dispersion of the glue in the synthetic rubber. The temperature is then reduced before the other compounding ingredients are added.

20 25

25

45

50

55

60

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

particular proportioning of the butadiene and acrylonitrile components of the copolymer.

I claim:

1. In a method of making textile fiber drafting elements employing a matrix of butadiene-acrylonitrile synthetic rubber which is deficient in lap resistance, the improvement which comprises heating said deficient synthetic rubber in an uncompounded condition to a temperature between 250° F. and 375° F. in the presence of oxygen while mechanically working the synthetic rubber to expose substantially all of it to oxygen while in a heated condition for an interval of between five and fifty minutes, sufficient to substantially improve the lap resistance of said synthetic rubber, and thereafter compounding the synthetic rubber so treated, forming the same into a textile fiber drafting element, and vulcanizing the same.

2. In a method of making textile fiber drafting elements employing a matrix of butadiene-acrylonitrile synthetic rubber which is deficient in lap resistance, the improvement which comprises heating said deficient synthetic rubber in an uncompounded condition to a temperature between 250° F. and 375° F. in the presence of oxygen while milling the synthetic rubber to expose substantially all of it to oxygen while in a heated condition for an interval of between five and fifty minutes, sufficient to substantially improve the lap resistance of said synthetic rubber, and thereafter compounding the synthetic rubber so treated, forming the same into a textile fiber drafting element, and vulcanizing the same.

3. In a method of making textile fiber drafting elements employing a matrix of butadiene-acrylonitrile synthetic rubber which is deficient in lap resistance, the improvement which comprises

heating said deficient synthetic rubber in an uncompounded condition to a temperature between 250° F. and 375° F. in the presence of oxygen while milling the synthetic rubber to expose substantially all of it to oxygen while in a heated condition for an interval of between five and fifty minutes, sufficient to substantially improve the lap resistance of said synthetic rubber, thereafter compounding the synthetic rubber with an electrolyte while mechanically working the mass at a temperature in the order of 240° F., and subsequently forming the same into a textile fiber drafting element and vulcanizing the compounded heat-treated rubber.

15 4. In a method of making textile fiber drafting elements employing a matrix of butadiene-acrylonitrile synthetic rubber which is deficient in lap resistance, the improvement which comprises heating said deficient synthetic rubber in an uncompounded condition to a temperature of about 320° F. in the presence of oxygen while mechanically working the synthetic rubber to expose substantially all of it to oxygen while in a heated condition for an interval of about twenty-five 20 minutes, sufficient to substantially improve the lap resistance of said synthetic rubber, and thereafter compounding the synthetic rubber so treated, forming the same into a textile fiber drafting element, and vulcanizing the same.

25 RICHARD A. GARRETT.

References Cited in the file of this patent

UNITED STATES PATENTS

|    | Number    | Name      | Date          |
|----|-----------|-----------|---------------|
| 35 | 2,450,410 | Baymiller | Oct. 5, 1948  |
|    | 2,505,349 | Daly      | Apr. 25, 1950 |